

June 28, 1938.

A. A. McCORMACK

2,122,378

RESILIENT YIELDING MATERIAL

Filed Oct. 30, 1935



INVENTOR.

Alex A McCormack  
BY  
Spencer Hardman and F. J. F.  
ATTORNEYS

## UNITED STATES PATENT OFFICE

2,122,378

## RESILIENT YIELDING MATERIAL

Alex A. McCormack, Dayton, Ohio, assignor to  
General Motors Corporation, Dayton, Ohio, a  
corporation of Delaware

Application October 30, 1935, Serial No. 47,516

2 Claims. (Cl. 106—22)

This invention relates to refrigerating apparatus and more particularly to a resilient yielding material for acting as a seal between metal parts in a refrigerating system.

In refrigerating systems it is necessary at many points to provide a fluid tight sealing means to prevent the escape of refrigerant and lubricant from the refrigerating system or from one part of the system to another. Yielding, elastic, resilient materials like rubber, are well suited to make a fluid tight seal between metal parts, but in the case of rubber, the refrigerant and lubricant attack and deteriorate the rubber and in a relatively short time causes it to become unsatisfactory for most sealing purposes and ordinarily permits the seal to leak after a period of time.

It has been proposed to use a polymer of chloro-2-butadiene-1,3 as a seal between metal parts of refrigerating systems in the place of rubber or other elastic materials which might be used. However, I find that ordinary compounds containing this polymer are not well suited for refrigerating systems because they tend to swell or increase in dimensions considerably when in contact with the refrigerant and the lubricant in the refrigerating system and because they tend to disintegrate or partially dissolve in the presence of a refrigerant and lubricant.

It is an object of my invention to provide an improved yielding, resilient, elastic rubber-like material containing no rubber which will satisfactorily and permanently provide a resilient elastic seal between metal parts of a refrigerating system.

It is a more specific object of my invention to provide an improved yielding elastic rubberlike material containing no rubber which will satisfactorily and permanently provide a seal between metal parts of a refrigerating system containing a halo derivative of a hydrocarbon and particularly systems containing chloro fluoro derivatives of an aliphatic hydrocarbon such as difluorodichloromethane and tetrafluorodichloroethane.

Further objects and advantages of the present invention will be apparent from the following description, reference being had to the accompanying drawing, wherein a preferred form of the present invention is clearly shown.

In the drawing:

Fig. 1 is a view of the refrigerating system, partly diagrammatic, illustrating one form of seal embodying my invention; and

Fig. 2 is an enlarged sectional view of a shaft portion of a refrigerant compressor illustrating another seal embodying my invention.

Briefly, as a resilient seal between metal parts in a refrigerating system, containing a halo derivative of a hydrocarbon, I employ a compound containing the following substances in parts by volume:

|                                   | Parts |
|-----------------------------------|-------|
| Polymer of chloro-2-butadiene-1,3 | 100   |
| Light calcined magnesium oxide    | 10    |
| Zinc oxide                        | 10    |
| FF wood rosin                     | 2     |
| Channel black (carbon)            | 29    |

Referring now more particularly to the drawing, there is shown a refrigerating system generally designated by the reference character 20 containing a refrigerant such as difluorodichloromethane or tetrafluorodichloroethane and a lubricant such as a mineral base refrigerator oil 25 22 shown in the bottom of the crank case of a compressor 24. The compressor 24 is driven through its drive shaft 26 by an electric motor 28 for compressing the refrigerant and for forwarding the compressed refrigerant to a condenser 30 30 where the compressed refrigerant is liquefied and forwarded under the control of a suitable automatic valve 32 to an evaporating means 34 located within an enclosure 36 containing a medium to be cooled. Within the evaporating means 34 the refrigerant evaporates under a reduced pressure and is returned to the crank case of the compressor by conduit means.

The drive shaft to the compressor extends 40 through the wall 38 of the compressor which wall is provided with a bearing 40 for supporting one end of the drive shaft. This wall is also provided with a hollow boss 42 for receiving a shaft seal which prevents the escape of refrigerant and lubricant from the crank case of the compressor through the opening provided for the drive shaft. This seal also prevents the ingress of air into the crank case. This boss 42 is provided with an end plate 46, fastened to the boss by screws 48.

This end plate is provided with an annular sealing surface 50 with which the shaft seal cooperates to form a relatively rotating fluid tight joint to prevent the escape of refrigerant and lubricant 5 and to prevent the ingress of air.

The shaft seal is provided with an annular sealing ring 52 which surrounds the reduced outer portion 54 of the drive shaft 26. This sealing ring 52 is preferably made of a smooth long 10 wearing material which is provided with a conical recess which receives a wedge-shaped, resilient, elastic, rubberlike sealing ring 56 of a material hereafter to be disclosed. This wedge-shaped rubberlike sealing ring 56 is tightly wedged in 15 between the sealing ring 52 and the reduced portion 54 of the drive shaft 26 so as to form a fluid tight seal between the sealing ring 52 and the reduced portion 54 of the drive shaft 26. This is performed by a cup-shaped annular member 58 20 which surrounds the reduced portion 54 of the drive shaft 26 and holds one face and the adjacent portion of the outer periphery of the wedge-shaped rubberlike sealing ring 56 and also surrounds and rides upon the outer periphery of 25 the sealing ring 52. This cup-shaped annular member 58 has an integral flange which receives one end of a compression type coil spring 60. This coil spring 60 provides the force necessary 30 for the cup-shaped member to wedge the resilient elastic rubberlike ring tightly between the sealing ring 52 and the reduced portion 54 of the drive shaft 26 as well as to provide sufficient force to hold the sealing ring 52 in sufficiently tight sealing engagement with the sealing surface 50 35 upon the end plate 46.

The other end of the compression spring 60 is held by a disc or washer 62 which presses against a shoulder 64 formed between the reduced portion 54 and the bearing portion of the drive shaft 40 26. The wedging of the rubberlike wedge-shaped ring 56 between the sealing ring 52 and the reduced portion 54 of the drive shaft 26 causes the entire shaft seal to rotate with the shaft 26. This causes relative rotation between 45 the sealing ring 52 and the sealing surface 50.

In order to lubricate these relatively rotating sealing surfaces, I have provided a passage 66 for oil for lubricating the space containing the 50 shaft seal. While this passage 66 is intended for oil, it also permits the free access of refrigerant to this space. It will thus be seen that the rubberlike wedge-shaped ring 56 is exposed to the action of both refrigerant and lubricant. 55 It is well known that rubber deteriorates in the presence of oil and is also attacked by the ordinary refrigerants. I have also found that ordinary compounds of rubber substitutes also are unsatisfactory for such use in a refrigerating system since most of them are subject to considerable swelling which is sufficient to distort the ring 56 and to prevent its proper action.

I have, therefore, provided an improved ring 66 60 of a molded composition which will meet the conditions required for this service. This composition contains no rubber and will withstand immersion in oil at relatively high temperatures without disintegrating or increasing the dimensions more than 10%. It is not materially attacked by halo derivatives of hydrocarbons, particularly difluorodichloromethane or tetrafluorodichloroethane. This material has a hardness of between 65 and 75 according to the Shore 70 Scleroscope system of measurement. It is com-

pounded according to the following formula in parts by volume:

|                                       | Parts by volume | Percent by volume | Specific gravity | 5  |
|---------------------------------------|-----------------|-------------------|------------------|----|
| Polymer of chloro-2-butadiene-1, 3... | 100             | 66.2              | 1.24             |    |
| Light calcined magnesium oxide....    | 10              | 6.6               | 2.4              |    |
| Zinc oxide.....                       | 10              | 6.6               | 5.57             |    |
| FF wood rosin.....                    | 2               | 1.3               | 1.4              | 10 |
| Channel black.....                    | 29              | 19.2              | 1.75             |    |

The channel black is a grade of carbon black. However, ordinary carbon black or lamp black or even graphite may be substituted in the same proportions for the channel black with very little or no change in properties. This substance may be used for various types of gaskets and washers used in refrigerating systems containing halo derivatives of hydrocarbon and other uses. In the place of FF wood rosin, any equivalent resin may be used.

In Fig. 2, I have shown another form of seal having this same composition. In this modification, there is shown a wall 120 of a refrigerant compressor, preferably containing a lubricant and a halo derivative of a hydrocarbon as a refrigerant such as difluorodichloromethane or tetrafluorodichloroethane. This wall 120 is provided with a bearing 122 which supports one end of the compressor drive shaft 124 provided with a reduced portion 126 forming a shoulder 128 upon the drive shaft. Surrounding this reduced portion of the drive shaft is a bellows type of shaft seal which is enclosed within a hollow boss 130 provided with an outer ring 132 which clamps the fixed end plate 134 of the shaft seal to the wall of the compressor. This end plate supports one end of a flexible metal bellows 136 which surrounds the reduced portion 126 of the drive shaft 124. The other end of this bellows is provided with a sealing ring 138 of a good wearing material which is provided with a flange 140 which in turn supports one end of the compression spring 142 extending between the flange 140 and the fixed end plate 134 for resiliently urging the sealing ring 138 toward the shoulder 128 on the drive shaft 124.

Heretofore, in such a shaft seal, it has been customary to have the sealing ring bear directly against the shoulder upon the drive shaft. However, I have found that it is difficult to provide a hard, smooth, perfectly flat, concentric, wearing surface upon the shoulders of the shaft and I have therefore proposed a separate sealing ring 144 which is resiliently held in place by a resilient elastic rubberlike sealing ring 146 preferably of the same molded composition as specified in detail above for the improved sealing ring 56. I find that such a compound for use in connection with halide refrigerants is superior to any similar compound heretofore used. This rubberlike sealing ring extends around three sides of the annular metal ring 144 and fits tightly between the rings 144 and the reduced portion 126 of the drive shaft 124.

The metal seal ring 144 is preferably hardened and ground so that a perfectly smooth face is provided for mating with sealing surface 148 of the ring 146. This seal likewise is exposed to the action of refrigerant and lubricant and must therefore be of such a composition as will withstand the action of the particular refrigerants and lubricants used.

While the form of embodiment of the invention

as herein disclosed, constitutes a preferred form, it is to be understood that other forms might be adopted, all coming within the scope of the claims which follow.

5. What is claimed is as follows:

1. A resilient seal for refrigerating systems comprising a substance containing ingredients about in the following proportions by volume:

|                                       | Per cent |
|---------------------------------------|----------|
| 10. Polymer of chloro-2-butadiene-1,3 | 66.2     |
| Magnesium oxide                       | 6.6      |
| Zinc oxide                            | 6.6      |
| Wood rosin                            | 1.3      |
| Carbon                                | 19.2     |

2. A resilient material comprising a substance containing ingredients about in the following proportions by volume:

|                                   | Parts |
|-----------------------------------|-------|
| Polymer of chloro-2-butadiene-1,3 | 100   |
| Magnesium oxide                   | 10    |
| Zinc oxide                        | 10    |
| Wood rosin                        | 2     |
| Carbon                            | 29    |

ALEX A. McCORMACK